

Sept. 3, 1940.

F. J. J. STOCK

2,213,827

TREATMENT OF PHOTOGRAPHIC FILMS

Filed Jan. 25, 1938



Inventor:  
FRIEDRICH JOHANN JAKOB STOCK

By:

Richards & Geier  
Attorneys:

## UNITED STATES PATENT OFFICE

2,213,827

## TREATMENT OF PHOTOGRAPHIC FILMS

Friedrich Johann Jacob Stock, Berlin, Germany

Application January 25, 1938, Serial No. 186,799  
In Germany September 23, 1936

2 Claims. (Cl. 95—2)

This invention relates to a method of treating photographic colour films of the kind comprising a carrier film, a plurality of superposed image layers and separating layers between the adjacent image layers, and to a colour film treated in accordance with this process.

It is an object of this invention to improve the luminosity and transparency of fresh or used colour films of this kind by changing substantially the mechanical state of the superposed image and separating layers and without acting upon the dye-stuff proper which is incorporated in the image layers.

Another object of my invention is to remove the separating layers which after the film has been dyed do not have any useful function but impair the brilliance of the colours and increase the distance between the superposed layers which for optical reasons should be as small as possible.

Still another object of the invention is to remove the detrimental effect of the irregular surfaces of the cavities which are formed in the image layers as the silver grains are removed in the photographic treatment, and tend to refract the light transmitted through the film.

According to this invention, the film is treated with a liquid, mixture of liquids or solution, which is capable of swelling the image layers to a degree nearly causing said image layers to adopt a sol condition. This state is hereinafter called "maximum swelling" for the purpose of this specification. The liquid moreover comprises substances adapted to dissolve or to dialyze through, the separating layers of the film. Thus the liquid penetrates through all separating layers down to the innermost image layer, whereby the irregular bounding surfaces of the cavities in the image layers are superficially converted to a sol and smoothened. Moreover, where solvents for the separating layers are used, the separating layers are dissolved in the treatment with the liquid and absorbed by the adjacent swollen image layers. The cavities in the image layers are at least partly filled up by the solid substances contained in the dissolved adjacent separating layers and/or dispersed or dissolved in the liquid which has been used for the treatment.

A schematical cross section of a colour film of the kind with which this invention is concerned, before and after the treatment, has been illustrated by way of example and schematically in the accompanying drawing.

Referring now to the drawing, prior to the treatment the carrier layer 1 of the film, consisting of celluloid, carries a preparatory layer 2 of any suitable material adapted to facilitate the adhesion of the following layers, viz:

An innermost image layer 3, preferably representing the blue-green colour layer, a separating layer 4, a second image layer 5, preferably repre-

senting the magenta colour layer, a second separating layer 6, and a third or exterior image layer 7, preferably representing the yellow colour layer

It will be understood that the separating layers 4 and 6 are merely provided, in the manner known per se, in order to prevent the substance used in the dyeing process for causing the layer 5 to adopt a red colour, from affecting the layer 3, or in order to prevent the substance used in the dyeing process to dye the yellow layer 7 from affecting the layers 5 and 3, respectively. Therefore, after the dyeing process, these separating layers or "blocking layers" not only do not serve any useful purpose but are positively harmful to the luminosity of the colours, the transparency of the film and sharpness of the contours. Some of the hollows or cavities produced by the removal of the silver grains are indicated at 8 and it will be seen that the cavities have very irregular contours causing undesirable refraction of the light transmitted through the film. Of course, the cavities 8 have been shown exaggerated both in scale and shape.

Now, after the treatment, the celluloid layer 1 and the layer 2 have remained substantially unchanged except that the separating line between the layers 2 and 3 is less sharp and distinct, due to the swelling action to which the layer 3 has been subjected. On the other hand, the separating layers 4 and 6 have disappeared entirely and the image layers 3, 5 and 6 lie directly adjacent to, and slightly intermeshing with, each other. The cavities 8 are now quasi "molten" into smooth globular shape and substantially filled by solid matter originating from the adjacent dissolved separating layers 4 and 6, respectively, and/or from the liquid which has been used for the treatment. Moreover, in the manner which will be hereinafter described, a further layer forming a hard surface coating has been deposited at 9, forming an intimate joint with the uppermost image layer 7. Thus, a substantially homogeneous layer is formed by the layers 2, 3, 5, 7, 9 which have intimately "grown together", due to the swelling and dissolving action to which these layers have been subjected.

Where the image layers consist of gelatine, the liquid which is used in the treatment of the film comprises substances causing swelling of the gelatine or solvents for gelatine suitably diluted to obviate complete solution of the gelatine. Fundamentally the desired effect is already produced by the exclusive use of a dilute acid or equivalent means such as potassium hydroxide or sodium hydroxide solution, in that with maximum swelling of the gelatine image layers 3, 5, 7, the rough edges of the tiny hollows in the interior of the layers are transformed to a smooth form. Since however acids or caustic alkalies alone or in combination with water destroy the colours, or at

least give rise to a change in the colours or make them run, the system of substances according to the invention comprises neutralized or naturally neutral solutions or liquids.

- 5 A mixture according to the invention may for instance consist of approximately equivalent proportions of dilute ammonia and dilute acetic acid, the dilutions being effected with water (neutral ammonium acetate solution) or of aqueous ammonium or sodium salicylate solution or of aqueous or alcohol-aqueous chloral hydrate solution. While this portion of the mixture serves for swelling the mixture, the mixture may furthermore comprise a chlorinated aliphatic alcohol of suitable strength in connection with non-chlorinated aliphatic alcohols or their derivatives, in order to dissolve the intermediate or blocking layers.
- 10 According to a further feature of the invention a dissolved colloid which is soluble to a sufficient extent in the mixture in question, advantageously primary acetyl cellulose, may be applied in the same operation or in succession. Thus, after the solvents have been evaporated, a multi-colour image layer 3, 5, 7, as per Figure 2 is formed which is hard at its surface, but elastic, perfectly homogeneous, and wherein the blocking layers 4 and 6 (Figure 1) have been dissolved and sucked up or absorbed by the adjacent image layers 3, 5, 7.
- 15 25 30 A preferred mixture which may be used in my novel process analyzes as follows:

| Parts by volume                                    |    |
|----------------------------------------------------|----|
| Aqueous sodium salicylate solution of 10% strength | 35 |
| Chlorinated ethyl alcohol                          | 30 |
| Amyl alcohol                                       | 3  |
| Ethyl alcohol                                      | 10 |
| Methyl alcohol                                     | 15 |
| Solactol (lactic acid ethyl ester)                 | 5  |
| Triacetin (poly-glycerine derivative)              | 2  |

In this mixture 1 part by weight of primary acetyl cellulose or cellulose triacetate may be dissolved or the film may be subjected to an after-treatment with a mixture of

|                                             |                 |     |
|---------------------------------------------|-----------------|-----|
| Water                                       | parts by volume | 30  |
| Chlorinated ethyl alcohol                   | do              | 30  |
| Methylene chloride or chlorinated methylene | do              | 38  |
| Triacetyl cellulose                         | parts by weight | 1-2 |

It will be understood that the substances hereinbefore stated by way of example may be substituted by equivalent substances causing the same effects and that the percentages may be varied according to the properties of the film material to be treated. For instance, diacetone alcohol may be used instead of lactic acid ester.

The solid substances which are dissolved in the liquid for the treatment of the film, for instance, colloids, should have substantially the same index of refraction as the image layers in order to prevent detrimental optical effects by the cavities in the image layers filled up by these solid substances.

The treatment of the colour film may be effected by applying the mixture to the film surface or by passing the film through a bath of the mixture. The former has been found more reliable and advantageous. According to the invention the improving process can to a certain extent be undertaken in steps at intervals. The image layer of the colour film is in this case first treated with the mixture according to the invention while the subsequent imbibition proceeds

gradually in a time spread over several days. Such a method permits accurate dosing of the substances to be employed in combination with a suitable colloidal suspension penetrating the surface and hardening it.

It is also possible to proceed by putting the mixture into a solution of low viscosity of for instance gelatine or agar-agar and then in a further stage of the process closing this to the outside with a coating of a material having a higher mechanical resistability than the image layers, for example cellulose esters, highly polymerised colloids, or the like forming a homogeneous combination with the top layer of the film and being impermeable or repellent to water, such as indicated at 9 in Figure 2.

Where the image layers consist substantially of gelatine, the liquid for the treatment of the film may preferably contain an aqueous solution of a neutral swelling agent for the gelatine, such as, for instance, salicylic acid, salicylate, benzene sulphonic acid salts or chloral hydrate either alone or in suitable mixture.

I contemplate, moreover, to add to the liquid used in my novel process for the treatment of the film, substances adapted to change the superficial tension between the film material and the liquid and to increase the adhesion between the film and the liquid, such as, for example, a colloid dispersion with water as a dispersing medium, whereby the liquid used in the treatment will more readily penetrate into the film and act upon the same in the desired manner.

A colour film treated in accordance with the invention exhibits improvement in regard to the clarity of the colour images and increased transparency.

I claim:

1. The process of treating a color film consisting of a plurality of superimposed gelatine layers containing subtractive dye images, said layers being separated by other gelatine layers softer than said image layers, which consists in subjecting said film to the action of a neutral agent which has a swelling effect upon said image layers and a dissolving effect upon said separating layers in such manner and for such time as to cause said separating layers to be absorbed and taken up by the adjacent gelatine image layers, with the result that said layers will join directly together with elimination of said separating layers, said absorption and dissolution causing said separating layers to fill up the interstices left by the removal of the sensitive silver salts.

2. The process of treating a color film consisting of a plurality of superimposed gelatine layers containing subtractive dye images, said layers being separated by other gelatine layers softer than said image layers, which consists in subjecting said film to the action of a neutral agent which has a swelling effect upon said image layers and a dissolving effect upon said separating layers in such manner and for such time as to cause said separating layers to be absorbed and taken up by the adjacent gelatine image layers, with the result that said layers will join directly together with elimination of said separating layers, said absorption and dissolution causing said separating layers to fill up the interstices left by the removal of the sensitive silver salts, said dissolution and swelling resulting from the use of a solution containing alkyl fatty acid esters.